

# UNITED STATES PATENT OFFICE.

FRANK D. CARNEY AND LEWIS B. LINDEMUTH, OF BETHLEHEM, PENNSYLVANIA.

## MANUFACTURE OF STEEL.

1,223,030.

Specification of Letters Patent. Patented Apr. 17, 1917.

No Drawing.

Application filed November 20, 1916. Serial No. 132,399.

*To all whom it may concern:*

Be it known that we, FRANK D. CARNEY and LEWIS B. LINDEMUTH, both citizens of the United States of America, and residents 5 of Bethlehem, Northampton county, Pennsylvania, have invented certain new and useful Improvements in the Manufacture of Steel; and we do hereby declare the following to be a full, clear, and exact description 10 of the invention, such as will enable others skilled in the art to which it appertains to make and use the same.

This invention relates to the manufacture 15 of steel by the duplex process, namely, where the pig iron is first treated in a Bessemer converter, and then treated under basic conditions in a basic lined open hearth, or equivalent, furnace for further purification. The steel is then run into ingot molds, and 20 the ingots suitably treated and manufactured into commercial rolled shapes.

There has been much difficulty in producing 25 these commercial shapes, as rails and other rolled shapes, free from such flaws as seams or small cracks when made of duplex steel, and we have found that often the cause of these flaws may be traced back to conditions occurring in the open hearth furnace, in even the most approved open-hearth 30 practice when treating bessemerized iron.

The object of this improvement in the 35 practice is to prevent the breaking and cracking of the ingot surfaces during rolling, and to produce a finished product more free from the defects known as "seams."

Of course, the outer surface of the ingot 40 may be removed, but this entails, in addition to the loss of metal that has no value beyond that of scrap metal, also the cost of labor, and the expense due to loss of heat.

We have found that it is most desirable 45 to overcome these defects by giving the metal more perfect casting properties or characteristics, so that these imperfections are not liable to occur from the quality of the steel, and we have done this with marked success.

We have discovered that a large part of 50 the surface defects in the finished metal may be prevented by carrying during the whole of the refining process a slag in the basic open hearth furnace with a sufficient content of manganese oxid, that manganese may be reduced from the slag and enter the 55 metal in the open hearth furnace, so that such metal will at all times during the re-

fining process in the basic open hearth furnace, contain in the neighborhood of .18% manganese, and preferably .20% or over. To obtain this condition during the refining 60 process the slag in the basic open hearth furnace must contain not less than 10.0% manganese oxid.

It is known that in the duplex process manganese in the pig iron charged into the 65 Bessemer converter, is eliminated early in the blow, except where such iron contains from three to five per cent. manganese, which is not a condition existing in this country, nor any place, except, perhaps, Sweden and 70 Norway.

The charge then to the open hearth furnace, which is entirely blown metal from a Bessemer converter, excepting ore, alloy and other necessary furnace additions, will contain from a trace to .05% manganese. Such a charge will not produce a steel of the best rolling qualities for, as we have found, both the slag and bath of metal have had their manganese content depleted. Such a condition will allow iron oxid to be formed from the bath of metal, and to enter the bath, giving the steel an appreciable percentage of this oxid, which in turn destroys 75 to a certain extent the good rolling qualities 80 of ingots cast from it.

It is known, and has always been customary, in the manufacture of steel by any process, to add manganese at the finish of the process either in the furnace or ladle or both, to give the steel the proper rolling qualities. This manganese is added, sometimes in conjunction with ferro-silicon, aluminum, ferro titanium, or other deoxidizing elements, to deoxidize the metal after it has been refined.

By our method of making up a slag in the basic open hearth furnace for refining bessemerized iron, the slag is saturated with manganese oxid to an extent that manganese reduces from the slag and passes into the metal of the bath, and oxidation of iron in the bath, or absorption of oxid by the bath, is prevented by the residual manganese in the bath which has a greater affinity for oxygen than iron. When the charge in the open hearth furnace is ready to be tapped, the residual manganese will be 0.18% to 0.30% with a slag of 10% manganese oxid, or higher, if a greater percentage of manganeseous materials have been added and the slag volume remains constant. 110

To obtain such a percentage of residual manganese in the open hearth metal we have found that it is necessary to form a slag that will analyze at least 10% manganese oxid.

- 6. In order to obtain such a slag and such an open hearth metal, we introduce into the open hearth furnace either before or with the charge, or during the refining stage, manganese materials, such as ferro-manganese or manganese ore, preferably the latter, in sufficient quantity to produce a slag having the manganese content above-mentioned; a part of the manganese will then be reduced by the usual reactions from the slag 10 and enter the metal bath below it in a quantity sufficient to prevent a great part of the oxidation of iron in the bath provided the manganese content of the slag is at least 10% manganese oxid. The surfaces of the 15 ingots produced by our process are more free from imperfections, and the surfaces of blooms rolled from the ingots, and the finished products rolled from the blooms are appreciably more free from imperfections, uniformly indicating the beneficial results 20 of the prevention of absorption of oxid by the metal of the bath during the refining process. We believe we are the first to apply this method of preventing the absorption of 25 oxid in the basic furnace treatment of bessemerized iron.

We claim—

- 1. The method of making duplex steel, which comprises charging bessemerized metal 30 into a basic open hearth furnace with sufficient manganese bearing material to produce a slag under basic conditions whose

manganese content is sufficiently great to permit a reduction of a portion of said manganese content and cause its entrance into 40 and its retention in the metal of the bath beneath it.

2. The method of making duplex steel, which comprises charging bessemerized metal into a basic open hearth furnace, then charging 45 sufficient manganese bearing material to produce a slag under basic conditions whose manganese content is sufficiently great to cause a portion of its manganese to enter the metal beneath it, and causing the metal 50 of the bath to contain at least 0.15% manganese during the entire refining operation.

3. The method of making duplex steel, which comprises charging bessemerized metal, into a basic open hearth furnace with sufficient 55 manganese material to produce a slag under basic conditions having a content of manganese oxid of ten per cent. or over.

4. The method of making duplex steel, which comprises charging bessemerized metal 60 into a basic open hearth furnace with manganese ore sufficient to produce a slag containing about ten per cent. manganese oxid under basic conditions existing in the furnace.

In testimony that we claim the foregoing as our invention, we have signed our names in presence of two subscribing witnesses.

FRANK D. CARNEY.  
LEWIS B. LINDEMUTH.

Witnesses:

E. D. HAEHNLE,  
R. M. BIRK.